

Feb. 28, 1928.

1,660,925

R. JARDINE

MOTOR VALVE AND ALLOY STEEL THEREFOR

Filed Jan. 3, 1922



Inventor  
Robert Jardine  
By *Gillson* *Gillson*  
Attorneys

Patented Feb. 28, 1928.

1,660,925

# UNITED STATES PATENT OFFICE.

ROBERT JARDINE, OF CHICAGO, ILLINOIS, ASSIGNOR TO RICH TOOL COMPANY, OF CHICAGO, ILLINOIS, A CORPORATION OF MAINE.

## MOTOR VALVE AND ALLOY STEEL THEREFOR.

Application filed January 3, 1922. Serial No. 526,667.

The invention relates to valves for explosive engines, and specially to poppet valves, wherein the valve head and adjacent portion of the stem are exposed to the high 5 temperature and corrosive action of the exploded charges and the rim or shoulder of the valve head is subjected to mechanical wear while highly heated. The object of the invention is to provide an improved 10 motor valve designed to resist both corrosive action and mechanical wear at high temperatures. A further object of the invention is to provide an alloy steel of novel composition from which the improved valve 15 may be produced.

The accompanying drawing is a side elevation showing a form of motor valve to which the invention may be applied.

As is well known, motor valves of the 20 form shown, especially exhaust valves, become highly heated in service, particularly in the head 10 and the adjacent portion 11 of the stem 12. These valves are accordingly exposed to the deteriorating influence 25 of both mechanical wear and the corrosive action of the exhaust gases, while in a heated condition. Furthermore, the effect of these two deteriorating influences is most pronounced upon the beveled rim or shoulder 30 13 of the valve head, where an accurate engagement with the valve seat (not shown) is desired.

It has also been recognized that warping of the valve, whether resulting from a temporary distortion due to unequal heating of different parts of the valve, or from a permanent distortion arising from repeated heating and cooling, disadvantageously affects the fit of the beveled shoulder 13 upon its seat. In this connection it is understood that warping does not occur to a noticeable degree from either of these causes, if the temperatures attained are not higher than the decalescent point of the steel from which the valve is made. It follows that objectionable warping is substantially avoided by forming the valve of a steel having a decalescent point which is above that likely to be attained in any part of the valve in service.

The present invention accordingly contemplates a valve which is formed from a special alloy steel, the same being preferably used for the rim portion 13 of the valve head 10, either with or without the forma-

tion of any part or all of the remainder of the valve from the same material. For this purpose the said special alloy steel should have as its important characteristics, so-called red hardness, a decalescent point 60 above the highest temperature likely to be attained in any part of the valve in service, and resistance to corrosion at high temperatures as well as in the cold state, to a marked degree. Such an alloy steel should 65 preferably contain chromium or chromium and silicon together, or its or their equivalents, in sufficient quantity to impart the desired resistance to corrosion. Likewise the said special alloy steel should contain 70 tungsten or tungsten and molybdenum together, or its or their equivalents, in sufficient quantity to impart the desired red hardness property.

Examples of the alloy steels which may 75 be used are as follows, the first being preferably employed for high grade valves adapted for use in so-called high-speed motors where high temperatures are attained and other service conditions are severe, although 80 it has been found that the second analysis indicated below gives excellent results.

### Alloy steel No. 1

|            | Per cent. | 85      |
|------------|-----------|---------|
| Carbon     | 1.00      | — 1.20  |
| Chromium   | 13.00     | — 15.00 |
| Tungsten   | 5.00      | — 7.00  |
| Molybdenum | .80       | — 1.00  |
| Silicon    | 2.00      | — 2.50  |
| Manganese  | .40       | — .60   |
| Phosphorus | .035 max. |         |
| Sulphur    | .035 max. |         |

### Alloy steel No. 2

|            | Per cent. | 95     |
|------------|-----------|--------|
| Carbon     | .50       | — .70  |
| Chromium   | 6.75      | — 7.75 |
| Tungsten   | 2.00      | — 3.00 |
| Molybdenum | .80       | — 1.00 |
| Silicon    | 2.00      | — 2.50 |
| Manganese  | .40       | — .60  |
| Sulphur    | .035 max. |        |
| Phosphorus | .035 max. |        |

The foregoing examples are merely illustrative and are not intended to indicate the maximum and minimum amounts of the various constituents within the scope of the invention. For example, there is no reason to believe that resistance to corrosion would become less if more than fifteen per cent of 105 110

chromium were used, and possibly a red hardness sufficient for some purposes would result from the use of less than two per cent of tungsten and eight-tenths of one per cent of molybdenum. On the other hand, while it is believed that an increased amount of chromium may be used without high silicon and a larger amount of tungsten used without molybdenum, it is understood that high silicon will not impart the desired resistance to corrosion unless a substantial amount of chromium is also used. Furthermore, molybdenum is desirably used for the reason that in the presence of tungsten it increases the red hardness property to a greater extent than an equal additional amount of tungsten, and it also avoids waste by reducing the tendency to piping and the like. Any of

the elements, usually regarded as scavaging or purifying elements, such as aluminum, 20 titanium, uranium, vanadium and zirconium, may be used in addition to manganese, if desired.

I claim as my invention—

An alloy containing the following:

|            | Per cent. |
|------------|-----------|
| Carbon     | 1.00      |
| Chromium   | 13.00     |
| Tungsten   | 5.00      |
| Molybdenum | .80       |
| Silicon    | 2.00      |
| Manganese  | .40       |
| Phosphorus | .035 max. |
| Sulphur    | .035 max. |

Remainder principally iron.

ROBERT JARDINE.